

# UNITED STATES PATENT OFFICE.

FRANZ SCHERHAG, OF VIENNA, AUSTRIA-HUNGARY.

## PROCESS OF MAKING PRIMINGS (COATINGS) FOR TRANSPARENCIES OR THE LIKE.

SPECIFICATION forming part of Letters Patent No. 712,728, dated November 4, 1902.

Application filed July 31, 1901. Serial No. 70,426. (No specimens.)

*To all whom it may concern:*

Be it known that I, FRANZ SCHERHAG, artist painter, a subject of the Emperor of Austria-Hungary, residing in XV Mariahilferstrasse 170, Vienna, Austria-Hungary, have invented a Process of Making a Priming (Coating) for Transparencies or the Like; and I do hereby declare the following to be a full, clear, and exact description of the invention, such as will enable others skilled in the art to which it appertains to make and use the same.

The subject of the present invention is a process for making a priming (coating) for the production of translucent pictures as a substitution for glass-paintings or transparencies, such as can be used for room or window decorations, translucent posters, (placard-bills,) advertisement-boards, for window-settings, for materials for Chinese lanterns, &c. Adaptable for this purpose is a thin threaded tissue with large meshes—such as muslin, book-muslin, cambric, &c., made out of silk, cotton, linen, &c.—stretched in a frame for preparation. This tissue receives a first coating of a solution of Russian glue in water, being applied in as hot a condition as possible. After becoming dry a second coating with a solution of gelatin, dextrine, (artificial gum,) or glycerin, and wood-vinegar in water is applied on the tissue and left to dry. The following solutions have proved to be suitable for the purpose: for the first solution, one hundred parts of water, twenty-five parts of Russian glue. For the second solution, one hundred parts of water, twenty-five parts of gelatin, four parts of dextrine, (artificial gum,) or glycerin, two parts of wood-vinegar. A hot coloring composition of chrome can be added to the last-named solution to render the glue and the glycerin insoluble in water. The result is that the spaces

between the threads are after the drying filled out with a translucent coat adaptable to be painted thereon with anilin water-colors, 45 (anilin colors soluble in water.)

A black oil-color or india-ink can be used to make the outlinings.

The priming being supplied with the painting, which can be done by hand or printed 50 thereon, it is covered with linseed-oil varnish, (dry oil,) copal, or damar-lac varnish, making thus the painting insensible to moisture, rain, &c., and allows a wet cleaning of the same.

Instead of the above-stated coating, especially for cheap priming, the stretched stuff mentioned can be covered with linseed-oil varnish. The painting is then applied on the priming and secured against humidity through the lac-varnish cover above stated. 60

Having now particularly described and ascertained the said invention and in what manner the same is to be performed, I declare that what I claim is—

The process of treating an open-mesh fabric so as to make the same suitable as a background for decorated objects which consists in first applying to said fabric a coating consisting of an adhesive substance, and then applying a coating consisting of a liquid translucent substance having water as its solvent and adapted to set to form a permanent coating filling the meshes of said fabric, said last-named coating having a chrome composition whose function is to impart color and insolubility to the material forming said coating, substantially as described. 75

In testimony that I claim the foregoing I have hereunto set my hand.

FRANZ SCHERHAG.

Witnesses:

ALBIN SCHILLER,  
ALVESTO S. HOGUE.